

May 23, 1933.

A. BERNSTEIN

1,910,879

PRODUCTION OF ARTIFICIAL FILAMENTS FROM VISCOSE SOLUTION

Filed July 11, 1929

*Fig. 1.*



*Fig. 2.*



Inventor:  
Arnold Bernstein  
By  
H. J. Helland  
His ATTORNEY

## UNITED STATES PATENT OFFICE

ARNOLD BERNSTEIN, OF MANNHEIM, GERMANY, ASSIGNOR TO ZELLSTOFFFABRIK,  
WALDHOF, OF MANNHEIM-WALDHOF, GERMANY

## PRODUCTION OF ARTIFICIAL FILAMENTS FROM VISCOSE SOLUTION

Application filed July 11, 1929, Serial No. 377,465, and in Germany July 13, 1928.

This invention relates to a method of and apparatus for producing artificial filaments from viscose solutions.

At the present time in the production of artificial filaments and the like from viscose solution in order to obtain goods fit for commercial use, the viscose solution is generally pressed through fine orifices into a precipitant which consists of a mixture of salts and acids. Good results are obtained, for example with a bath containing a considerable excess of neutral salts. The object in using such a precipitant is to exercise a mild action on the filament separating out in the acid liquid. Subsequently precipitation of the xanthogenate takes place followed immediately by a transformation into cellulose hydrate.

Such spinning baths, however, possess the disadvantage that salts and acids are present in an admixed state in one bath and that the action of the acids particularly when using high concentrations sets in very quickly after the introduction of the viscose into the precipitant. This results in decomposition of the viscose which strikes deep at a very early stage of the formation of the artificial filament which, amongst other things, renders a fine drawing out of the threads extraordinarily difficult.

Attempts have already been made to effect a separate action of salts and acids in which filaments separated out in pure salt solution are conveyed into other baths containing only acids or in which filaments withdrawn from pure salt baths are wound up on spools or the like which rotate in an acid bath. This manner of using separate baths is, however, not satisfactory as firstly strong adherence of the filaments to one another can easily take place, and secondly, the artificial filaments after action of a pure salt solution do not in general yet possess sufficient strength to endure the passage necessary on being transferred to another apparatus.

One object of the invention is to provide a method of producing artificial filaments wherein coagulation and fixation of the filaments take place in separate stages without damage to the filament on being transferred from one stage to the next.

Another object of the invention is to provide apparatus for forming artificial filaments wherein the filament may be transferred without damage from one part of the apparatus to another.

The invention is more particularly described with reference to the accompanying drawing forming part of this specification and showing apparatus adapted for carrying out the process. On the drawing:

Fig. 1 is a view, chiefly in cross-section, of apparatus in accordance with the invention; and

Fig. 2 is a top view of the apparatus shown in Fig. 1.

The apparatus comprises a precipitant vessel which is sub-divided by the wall *e* into two chambers A and B. *a* denotes the spinning nozzles, *f* and *f'* the inlet pipes for the salt solution and acid respectively, *g* and *g'* overflow conduits for the withdrawal of the salt solution and acid respectively out of the precipitant container. Filament guides *h* are provided over which the filaments *b* pass to the spooling devices *d*.

The spinning process may be carried out with this apparatus, for example in the following manner. At the end where the viscose solution enters a pure salt solution having for example, a 30% salt content is introduced into the vessel through pipe *f* and is withdrawn again through the overflow device *g* located somewhat centrally of the bath. The second part B of the vessel arranged behind this overflow device contains the acid, for example 30% sulphuric acid, which is introduced through the supply pipe *f'* shortly behind the overflow *g* for the salt solution and is again withdrawn at the end

of the precipitant container through the second overflow device  $g'$ .

The viscose solution is forced into the vessel through the nozzles  $a$  and coagulates 5 on its passage through the salt solution present in the part A. The filament is led over the partition within the body of said solutions and on its further passage through the second part of the vessel it is transformed into 10 cellulose hydrate and the filament is fixed by the action of the acid. In this manner of producing artificial filaments the cellulose filament is withdrawn at the end of the bath possessing greater strength so that it can 15 be led off without difficulty on suitable winding devices or the like. In order to prevent any dangerous after effect of the strong acid, the artificial threads are preferably caused, shortly after leaving the acid bath to be 20 washed with warm water or steam. If desired, instead of inorganic salts, suitable organic coagulating media can also be substituted in the first part A of the bath in order to produce the precipitation of the viscose.

25 Similarly, the method of operation above described can also be utilized in the production of films and like formations from viscose solution.

30 The improved process is particularly suitable for the production of very fine silk filaments as in this manner of forming the cellulose filament a very uniform and fine drawing out is rendered possible.

What I claim is:—

35 1. In apparatus for forming artificial tissues from viscose solution the combination of a vessel adapted to contain liquid, a partition of less height than said vessel dividing said vessel into two separate compartments, 40 means to introduce a precipitant at the outer end of one of said compartments, means to remove said precipitant from said compartment located adjacent and above the upper edge of said partition, means to introduce 45 an acid solution into said other compartment adjacent said partition, means to remove said acid solution from the opposite end of said second compartment and located above the upper edge of said partition, means to introduce 50 viscose solution into the outer end of said first compartment and means to draw the coagulated viscose body through said first and second compartments.

2. Apparatus for forming artificial filaments and the like from viscose solution comprising a single container, a partition within said container extending from the bottom thereof to a height less than the height of the walls of said container to divide said container into two substantially separate compartments adapted to form a precipitating bath and a fixing bath, means to introduce precipitant solution into said first compartment, means to remove said precipitant solution from said first compartment located

above the upper edge of said partition, means to introduce acid fixing solution into said second compartment and means to withdraw said fixing solution located at a level above the upper edge of said partition.

70 In testimony whereof I have affixed my signature.

ARNOLD BERNSTEIN.

75

80

85

90

95

100

105

110

115

120

125

130